

# United States Patent

[11] 3,617,268

[72] Inventors **Yoshinobu Murakami;**  
Kazuhisa Morimoto, both of Osaka, Japan  
[21] Appl. No. **4,200**  
[22] Filed **Jan. 20, 1970**  
[45] Patented **Nov. 2, 1971**  
[73] Assignee **Matsushita Electric Industrial Co., Ltd.**  
Kadoma, Osaka, Japan  
[32] Priority **Jan. 30, 1969**  
[33] **Japan**  
[31] **44/7501**

[54] **ELECTROPHOTOGRAPHIC MATERIALS**  
7 Claims, 6 Drawing Figs.

[52] **U.S. Cl.**..... **96/1.5,**  
..... **96/1.6**

[51] **Int. Cl.**..... **G03g 5/06**  
[50] **Field of Search.**..... **96/1.5, 1.6;**  
..... **252/501**

[56] **References Cited**  
UNITED STATES PATENTS

3,250,615 5/1966 Van Allan et al. .... **96/1.6 X**  
3,526,502 9/1970 Murakami et al. .... **96/1.5**

*Primary Examiner—Charles E. Van Horn*  
*Attorney—Wenderoth, Lind & Ponack*

**ABSTRACT:** A photosensitive material for electrophotography comprising an organic photoconductive compound and a sensitizer consisting of reaction products of a benzopyrylium salt and a benzopyrane.

PATENTED NOV 2 1971

3,617,268

SHEET 1 OF 2

FIG. 1.



FIG. 3.



FIG. 2.



INVENTOR

YOSHINOBU MURAKAMI  
KAZUHISA MORIMOTO

BY  
Wenderoth, Lind & Ponack  
ATTORNEYS

PATENTED NOV 2 1971

3,617,268

SHEET 2 OF 2

FIG. 4.



FIG. 5.



FIG. 6.



INVENTOR

YOSHINOBU MURAKAMI  
KAZUHISA MORIMOTO  
BY *Wenderoth, Lind & Ponack*  
ATTORNEYS

## ELECTROPHOTOGRAPHIC MATERIALS

This invention relates to an electrophotographic material and more particularly to a photoconductive insulating material comprising an organic photoconductive compound and a sensitizer.

Various photoconductive insulating layers are well known in the electrophotographic art for making copies of documents, drawings, transparencies, etc. These layers contain an organic photoconductive compound, such as poly-N-vinylcarbazole, poly-3,6-dibromo-N-vinylcarbazole, brominated poly-N-vinylcarbazole, nitrated poly-N-vinylcarbazole, polyacenaphthylene, etc. These layers are nonconductors of electricity before exposure and become electrical conductors upon exposure.

It is necessary for the electrophotographic art that the photoconductive insulating material has a high photoconductivity in the region of the visible spectrum. Such a photoconductive insulating material makes it possible for the electrophotographic art to employ inexpensive and convenient light sources such as incandescent lamps in a reduced exposure time and to reproduce colored pictures. The photoconductive compounds mentioned above, however, have usually a low photoconductivity and spectrum characteristics sensitive to the short wavelength region of the exposure light and do not satisfy entirely the above requirement.

It is known that an addition of a so-called sensitizer can improve photoconductivity and spectrum response of the above photoconductive compounds. Conventional sensitizers are dyestuffs, such as triarylmethane dyes, xanthene dyes, triazine dyes or acridine dyes, but the conventional sensitizers are not entirely satisfactory for improvement of the photoconductivity and the spectrum response of the available organic photoconductive compounds.

In addition to the high photoconductivity and spectrum response sensitive to visible light, the electrophotographic art requires a high electric resistance of photoconductive materials in the dark. Conventional sensitizers promote the photoconductivity but increase the dark conductivity. A high dark conductivity of photoconductive materials is not desirable because it results in a loss of the applied electrostatic charge in the dark.

## OBJECT OF THE INVENTION

An object of the invention is to provide electrophotographic materials having a high photoconductivity and spectrum response sensitive to visible light.

Another object of the invention is to provide electrophotographic materials having a high electric resistance in the dark.

## EXPLANATION OF FIGURES

These and other objects of the present invention will be apparent upon consideration of the following detailed description taken together with accompanying drawings wherein:

FIG. 1 represents the absorption spectra, in 1,2-dichloroethane, of one example (Sample Number 27) of sensitizers according to the present invention under comparison with those of 2-(p-methoxystyryl)-3-phenylbenzopyrylium perchlorate (Compound Number 2), in 1,2-dichloroethane, and 2-(p-methoxystyryl)-3-phenyl-4-methoxypyran (Compound Number 11) in methanol.

FIG. 2 represents the infrared absorption spectra in KBr method of Compound Number 2, 11 and Sample Number 27.

FIG. 3 represents the wedge spectrogram for an electrophotographic material coated with a solution containing 10 weight percent of brominated poly-N-vinylcarbazole and 0.02 weight percent of sensitizer (Sample Number 27), the brominated poly-N-vinylcarbazole being dissolved in a solvent consisting of 4 parts by weight of chlorobenzene and 1 part by weight of 1,2-dichloroethane under comparison with those of brominated poly-N-vinylcarbazole.

FIG. 4 represents the wedge spectrogram of an electrophotographic material coated with a 10 weight percent

solution of brominated poly-N-Vinylcarbazole sensitized with 0.02 weight % of Sample Number 50, the brominated poly-N-vinylcarbazole being dissolved in a solvent consisting of 4 parts by weight of chlorobenzene and 1 part by weight of 1,2-dichloroethane, under comparison with the wedge spectrogram of an electrophotographic material coated with a 10 weight percent solution of brominated poly-N-vinylcarbazole sensitized with 0.06 weight percent of Compound Number 9, which is the raw material of Sample Number 50, the brominated poly-N-vinylcarbazole being dissolved in a solvent consisting of 4 parts by weight of chlorobenzene and 1 part by weight of 1,2-dichloroethane.

FIG. 5 represents the wedge spectrogram of an electrophotographic material coated with a 10 weight percent solution of poly-N-vinylcarbazole sensitized with 0.03 weight percent of Sample Number 39, the poly-N-vinylcarbazole being dissolved in a solvent consisting of 4 parts by weight of toluene and 1 part by weight of 1,2-dichloroethane.

FIG. 6 represents the wedge spectrogram of an electrophotographic material coated with 10 weight percent solution of poly-N-vinylcarbazole sensitized with 0.03 weight percent of Sample Number 28, the poly-N-vinylcarbazole being dissolved in a solvent consisting of 4 parts by weight of toluene and 1 part by weight of 1,2-dichloroethane.

## SCOPE OF INVENTION

An electrophotographic material according to the present invention comprises a conductive support layer and a photoconductive insulating layer, the latter comprising a combination of an organic photoconductive compound and a sensitizer. Said organic photoconductive compound consisting essentially of at least one compound selected from the group consisting of poly-N-vinylcarbazole, poly-3,6-dibromo-N-vinylcarbazole, brominated poly-N-vinylcarbazole, nitrated poly-N-vinylcarbazole and polyacenaphthylene. Said sensitizer consisting essentially of at least one compound selected from the group consisting of reaction products of a benzopyrylium salt having a chemical formula A and a benzopyrone having a chemical formula B; the chemical formula A is



wherein R<sub>1</sub> is an aliphatic group such as styryl, p-methoxystyryl,  $\omega$ -phenylbutadienyl; aromatic group such as phenyl, p-methoxyphenyl;

R<sub>2</sub> is selected from the group consisting of hydrogen and phenyl radical;

R<sub>3</sub> is selected from the group consisting of hydrogen and methoxy radical;

Anion<sup>1</sup> is fluoborate, chloroferrate, chlorozincate or perchlorate anion.

The chemical formula B is



65

wherein R<sub>4</sub> is an aliphatic group such as styryl, p-methoxystyryl,

$\omega$ -phenylbutadienyl; aromatic group such as phenyl, p-methoxyphenyl;

R<sub>5</sub> is selected from the group consisting of hydrogen and phenyl radical;

R<sub>6</sub> is selected from the group consisting of hydrogen and methoxy radical.

Said reaction products can be formed by employing the following steps which comprise (1) providing a solution of said

benzopyrylium salt in a suitable solvent such as 1,2-dichloroethane, (2) providing a solution of said benzopyrane in a suitable solvent such as 1,2-dichloroethane, (3) mixing both solutions and heating the mixed solution (4) pouring the heated solution into a suitable precipitant such as ether to form a precipitate (5) separating the precipitate from the precipitant and (6) purifying the separated precipitate.

#### BENZOPYRYLIUM SALT

There have been known four methods for preparing the benzopyrylium salt. The first method is a modification of a method disclosed in J. Chem. Soc., 1935, page 941 and is based on the reaction of a phenol or phenol derivative with a  $\beta$ -dicarbonyl compound or an  $\alpha, \beta$ -unsaturated ketone in the presence of hydrogen chloride, sulfuric acid, ferric chloride, acetic or formic acid.

The second method comprises using an intermediate product prepared from a phenol and a coumarin derivative in the presence of phosphorus oxychloride or zinc chloride in a similar way to that disclosed in Helv. chim. acta, 34, page 1761 (1951).

The third method is based on a method disclosed in J. Chem. Soc., 74, page 3,445 (1952). A ring closure process of an o-hydroxybenzaldehyde and a carbonyl compound in the presence of an alkali forms a benzopyrylium ring. An ethenyl group of an active  $\alpha$ -methylene radical in the 2-position of 2-alkylbenzopyrylium has an important role on the benzopyrylium ring closure process.

The fourth method is based on a method disclosed in J. Chem. Soc., 1929, page 936 and is effected in one step by both ring closure and ethenylation of an o-hydroxybenzaldehyde with a carbonyl compound in the presence of an alkali.

Examples of suitable benzopyrylium salt are given in table 1 below.

TABLE 1

| Compound Number | Name of compound                                                                | Absorption maximum ( $\lambda_{\text{max.}} \text{ m}\mu$ ) in 1,2-dichloroethane |
|-----------------|---------------------------------------------------------------------------------|-----------------------------------------------------------------------------------|
| 1.              | 2-( $\alpha$ -isopropyl- $\omega$ -phenylbutadienyl)-benzopyrylium perchlorate. | 530                                                                               |
| 2.              | 2-(p-methoxystyryl)-3-phenylbenzopyrylium perchlorate.                          | 552                                                                               |
| 2B.             | 2-(p-methoxystyryl)-3-phenylbenzopyrylium fluoborate.                           | 560                                                                               |
| 2F.             | 2-(p-methoxystyryl)-3-phenylbenzopyrylium chloroferrate.                        | 560                                                                               |
| 2Z.             | 2-(p-methoxystyryl)-3-phenylbenzopyrylium chlorozincate.                        | 560                                                                               |
| 3.              | 2-(p-methoxystyryl)-3-phenyl-8-methoxybenzopyrylium perchlorate.                | 555                                                                               |
| 4.              | 2-(p-methoxyphenyl)-benzopyrylium perchlorate.                                  | 455                                                                               |
| 5.              | 2-(p-methoxyphenyl)-8-methoxybenzopyrylium perchlorate.                         | 460                                                                               |
| 6.              | 2-styryl-3-phenylbenzopyrylium perchlorate.                                     | 503                                                                               |
| 7.              | 2-( $\alpha$ -isopropyl-p-methoxystyryl)-benzopyrylium perchlorate.             | 543                                                                               |
| 8.              | 2-( $\alpha$ -isopropylstyryl)-benzopyrylium perchlorate.                       | 458                                                                               |
| 9.              | 2-phenylbenzopyrylium perchlorate.                                              | 410                                                                               |

Examples of reaction procedure to prepare a benzopyrylium salt are shown as follows:

#### 1. 2-(p-Methoxystyryl)-3-phenylbenzopyrylium perchlorate (Compound Number 2)

5 grams of salicylaldehyde and 5.5 grams of phenylacetone are dissolved in 15 milliliters of formic acid in order to obtain a solution and dry hydrogen chloride gas is slowly blown into the solution in an ice-cooled bath for 1.5 hour. After standing in an icebox for 3 hours the solution is added 6 grams of p-anisaldehyde and 25 milliliters of formic acid, then dry hydrogen chloride gas is slowly blown into the solution in an ice-cooled bath for 1 hour. After standing overnight at a room temperature, the solution in an ice-cooled bath has 90 milliliters of 10 percent perchloric acid added slowly thereto while being stirred. Precipitation starts when the perchloric acid is added to the solution. The precipitate obtained is filtered off, washed thoroughly with ether and recrystallized from an acetic acid to yield 7 grams of needle-crystal which has a melting point of 229° to 230° C.

2. 2-( $\alpha$ -Isopropylstyryl)-benzopyrylium perchlorate (Compound Number 8)

5 grams of 2-oxystyrylisobutyl ketone and 10 grams of benzaldehyde are dissolved in 100 milliliters of ether in order to obtain a solution and 15 grams of 60 percent perchloric acid is slowly added to the solution. Precipitation starts when the solution is saturated with dry hydrogen chloride gas. The solution and precipitate are then allowed to stand overnight in an icebox, and the resulting precipitate is collected by filtration, washed thoroughly with ether. The crude product obtained is recrystallized from a solvent consisting of 5 parts by weight of acetic acid and 1 part by weight of dichloroethane to yield 10 grams of crystal, having a melting point of 169° to 170° C.

Other benzopyrylium salts are obtained by similar procedures as stated above.

#### BENZOPYRANE

20 The benzopyranes are easily prepared by one of the following two methods. A first method is that benzopyrane is prepared by heating, under a reflux, a methanol solution of said benzopyrylium salt with sodium bicarbonate. A second method is that benzopyrane is prepared by heating an alcohol solution of said benzopyrylium salt with sodium hydroxide or potassium hydroxide.

25 Examples of suitable benzopyranes are given in table 2 below.

TABLE 2

| Compound Number | Name of compound                                                           | Absorption maximum ( $\lambda_{\text{max.}} \text{ m}\mu$ ) in methanol |
|-----------------|----------------------------------------------------------------------------|-------------------------------------------------------------------------|
| 10.             | 2-( $\alpha$ -isopropyl $\omega$ -phenyl butadienyl)-4-methoxybenzopyrane. | 300, 360                                                                |
| 11.             | 2-(p-methoxystyryl)-3-phenyl-4-methoxybenzopyrane.                         | 270, 360                                                                |
| 12.             | 2-(p-methoxystyryl)-3-phenyl-4,8-dimethoxybenzopyrane.                     | 260, 365                                                                |
| 13.             | 2-styryl-3-phenyl-4-methoxybenzopyrane.                                    | 260, 380                                                                |
| 14.             | 2-phenyl-4-methoxybenzopyrane.                                             | 260, 300                                                                |
| 15.             | 2-(p-methoxyphenyl)-4-methoxybenzopyrane.                                  | 260, 360                                                                |
| 16.             | 2-( $\alpha$ -isopropyl-p-methoxystyryl)-4-methoxybenzopyrane.             | 250, 360                                                                |
| 17.             | 2-( $\alpha$ -isopropylstyryl)-4-methoxybenzopyrane.                       | 250, 360                                                                |

45 Examples of reaction procedure to prepare a benzopyrane are shown as follows:

#### 3. 2-(p-Methoxystyryl)-3-phenyl-4-methoxybenzopyrane (Compound Number 11)

4 grams of 2-(p-methoxystyryl)-3-phenylbenzopyrylium perchlorate are dissolved in 800 milliliters of hot methanol in order to obtain a solution. Then, 10 grams of sodium bicarbonate is added to the cold solution. After the solution is refluxed for 10 minutes, the solution is cooled and a precipitate obtained is collected by filtration and washed with methanol. The filtrates are distilled by a rotary evaporator to yield a crude compound. The crude compound filtered off is dissolved in 500 milliliters of methanol under heating in order to obtain a solution, then, the solution is cooled, added 500 milliliters of water and allowed to stand overnight. The resulting precipitate having a melting point of 84° to 86° C. is then collected by filtration.

#### 4. 2-Styryl-3-phenyl-4-methoxybenzopyrane (Compound Number 13)

65 Similarly to the procedure as stated above, 2.5 grams of yellow crystal having a melting point of 63° to 66° C. is obtained from 4 grams of 2-styryl-3-phenylbenzopyrylium perchlorate.

Other benzopyranes are obtained by the similar procedure as stated above.

70 The benzopyrane thus obtained is unstable and tends to change to a benzopyrylium salt by adding organic acid or inorganic acid. Furthermore, the benzopyrane is colored by air. Therefore, an improved preparation procedure is developed as follows: In the preparation procedure such as procedure (3) or (4), the crude benzopyrane is not recrystallized from a methanol-water solution, but the crude compound is shaken in

a flask with a mixed solvent of 2 parts by weight of benzene and 1 part by weight of water. Then, a benzene solution containing yielded benzopyrane is separated from water and dried with sodium sulfate anhydrous. The benzene solution is distilled to yield a solid compound. The solid compound thus obtained is used as a raw material of benzopyrane.

## SENSITIZER

The sensitizer according to the present invention is produced by the reaction of a benzopyrylium salt and a benzopyrane. Examples of the reaction products are shown in table 3 with their physical properties.

TABLE 3

| Sample No. | Species           | M.P.<br>(°C.) | $\lambda_{max}$ (m $\mu$ )<br>in 1,2-dichloroethane |
|------------|-------------------|---------------|-----------------------------------------------------|
| Compounds: |                   |               |                                                     |
| 18         | No. 10 and No. 1  | 167~171       | 540, 670                                            |
| 19         | No. 10 and No. 2  | 138~141       | 580, 620                                            |
| 20         | No. 10 and No. 4  | 154~157       | 465, 670                                            |
| 21         | No. 10 and No. 5  | 158~162       | 455, 675                                            |
| 22         | No. 10 and No. 6  | 156~159       | 570, 680                                            |
| 23         | No. 10 and No. 7  | 167~171       | 685                                                 |
| 24         | No. 10 and No. 8  | 163~167       | 685                                                 |
| 25         | No. 10 and No. 9  | 181~184       | 545, 675                                            |
| 26         | No. 11 and No. 1  | 183~185       | 595, 625                                            |
| 27         | No. 11 and No. 2  | 162~165       | 595, 645                                            |
| 27B        | No. 11 and No. 2B | 150~154       | 595, 645                                            |
| 27E        | No. 11 and No. 2E | 118~119       | 595, 645                                            |
| 27Z        | No. 11 and No. 2Z | 176~179       | 595, 645                                            |
| 28         | No. 11 and No. 4  | 206~209       | 555, 595                                            |
| 29         | No. 11 and No. 5  | 168~171       | 550, 590                                            |
| 30         | No. 11 and No. 6  | 157~160       | 595, 700                                            |
| 31         | No. 11 and No. 7  | 138~140       | 500, 590                                            |
| 32         | No. 11 and No. 8  | 136~138       | 585, 650                                            |
| 33         | No. 11 and No. 9  | 157~161       | 545, 635                                            |
| 34         | No. 12 and No. 3  | 224~225       | 590, 640                                            |
| 35         | No. 13 and No. 1  | 159~163       | 630, 700                                            |
| 36         | No. 13 and No. 2  | 163~166       | 590, 640, 700                                       |
| 37         | No. 13 and No. 4  | 155~160       | 550, 593, 710                                       |
| 38         | No. 13 and No. 5  | 163~167       | 550, 590, 705                                       |
| 39         | No. 13 and No. 6  | 170~174       | 595, 640, 705                                       |
| 40         | No. 13 and No. 7  | 145~148       | 595, 705                                            |
| 41         | No. 13 and No. 8  | 139~142       | 588, 705                                            |
| 42         | No. 13 and No. 9  | 218~220       | 585, 705                                            |
| 43         | No. 14 and No. 1  | 126~129       | 610, 690                                            |
| 44         | No. 14 and No. 2  | 122~125       | 540, 580                                            |
| 45         | No. 14 and No. 4  | 118~121       | 610                                                 |
| 46         | No. 14 and No. 5  | 125~129       | 610                                                 |
| 47         | No. 14 and No. 6  | 136~140       | 540, 580                                            |
| 48         | No. 14 and No. 7  | 124~127       | 505, 610                                            |
| 49         | No. 14 and No. 8  | 113~116       | 610                                                 |
| 50         | No. 14 and No. 9  | 144~147       | 610                                                 |
| 51         | No. 15 and No. 2  | 151~154       | 550, 590                                            |
| 52         | No. 15 and No. 4  | 145~160       | 630                                                 |
| 53         | No. 15 and No. 6  | 131~135       | 530, 590                                            |
| 54         | No. 15 and No. 9  | 142~145       | 630                                                 |
| 55         | No. 16 and No. 2  | 156~160       | 560, 580                                            |
| 56         | No. 16 and No. 6  | 151~155       | 565, 685                                            |
| 57         | No. 16 and No. 7  | 116~119       | 690                                                 |
| 58         | No. 16 and No. 9  | 124~127       | 515                                                 |
| 59         | No. 17 and No. 2  | 112~116       | 550, 585                                            |
| 60         | No. 17 and No. 6  | 128~131       | 585, 680                                            |
| 61         | No. 17 and No. 8  | 83~87         | 555, 690                                            |
| 62         | No. 17 and No. 9  | 118~122       | 590                                                 |

The formation of sensitizer according to the present invention is accomplished by heating a solution of the benzopyrylium salt and benzopyrane in a suitable solvent such as dichloroethane at 40° to 70° C. for several hours to dozens of hours. The amount of benzopyrane to be used is one to three times by molar weight of benzopyrylium salt to be used. The color of the solution changes to dark color with a progress of the reaction. For example, FIG. 1 shows the absorption spectra of, Compound Number 2 (in dichloroethane) and Compound Number 11 (in methanol), and reaction product, Sample Number 27 (in dichloroethane). When Compound Number 2 (reddish violet) reacts with Compound Number 11 (pale yellow), the color of the reacting solution changes from reddish violet to blue. After the completion of the reaction, the solution is poured into ether to obtain a crude product. The crude product is dissolved in dichloroethane, then, the solution is poured into ether to yield a pure reaction product. As shown in FIG. 2 at the spectrum of Sample Number 27, the infrared absorption bands 1,478, 1,375 and 975 cm<sup>-1</sup> are distinguished as compared with Compound Number 2.

Some examples of methods of preparing the sensitizer are set forth below in accordance with table 3. It will be apparent

5

to those skilled in the art that other sensitizers according to the present invention may be prepared by methods similar to those described in general hereinabove and specifically herein below.

6

## I. Sample Number 26

3.6 grams of Compound Number 11 and 2.0 grams of Compound Number 1 are dissolved in 40 milliliters of 1,2-dichloroethane which is purified to eliminate an acidic material by sodium carbonate. A so-obtained solution is stirred at 50° C. for 5 hours. The color of the solution is red at the beginning of the reaction, but, the color changes in accordance with the reaction progress. At the end point of the reaction the color of the solution is blue. After the completion of the reaction, the solution is cooled to 24° C. and poured into 300 milliliters of ether to yield a precipitate. The precipitate is washed thoroughly with ether, dried and dissolved in dichloroethane to obtain a solution. The solution is poured into ether to yield 2.5 grams of crystal having a melting point of 183° to 185° C.

## II. Sample Number 39

3.4 grams of Compound Number 13 and 2 grams of Compound Number 6 are dissolved in 75 milliliters of 1,2-dichloroethane which is purified to eliminate an acidic material. A so-obtained solution is stirred at 50° C. for 8 hours. After the same procedure as stated in (I), 3 grams of crystal is the yield. The crystal has a melting point of 170° to 174° C. and a solution of the crystal in 1,2-dichloroethane is green.

## III. Sample Number 50

4.8 grams of Compound Number 14 and 3 grams of Compound Number 9 are dissolved in 80 milliliters of pure 1,2-dichloroethane to obtain a solution. The solution is stirred at 50° C. for 8 hours. The same procedure as stated in (I) yields 5 grams of crystal. The crystal has a melting point of 144° to 147° C. and a solution of the crystal in 1,2-dichloroethane is blue.

## IV. Sample Number 52

2.7 grams of Compound Number 15 and 1.7 gram of Compound Number 4 are dissolved in 40 milliliters of pure 1,2-dichloroethane to obtain a solution. The solution is stirred at 50° C. for 20 hours, during which the color of the solution changes from orange to green. After the same procedure as stated in (I), 3 grams of crystal is the yield. The crystal has a melting point of 145° to 150° C.

## PHOTOCONDUCTIVE INSULATING MATERIAL

An improved photoconductive insulating material adapted for aforesaid photoconductive insulating layer can be obtained by a combination of aforesaid sensitizer and aforesaid organic photoconductive compound selected from the group consisting of poly-N-vinylcarbazole, poly-3,6-dibromo-N-vinylcarbazole, brominated poly-N-vinylcarbazole, nitrated poly-N-vinylcarbazole and polyacenaphthylene. The sensitizer according to the present invention is usually added to a solution of the photoconductive compound in the form of a solution in a suitable solvent, such as dichloroethane, methylene chloride, chloroform, or a combination thereof. An added amount of said sensitizer is from 0.005 gram to 0.02 gram, preferably from 0.0015 gram to 0.015 gram with respect to 1 gram of said organic photoconductive compound.

Poly-3,6-dibromo-N-vinylcarbazole and brominated poly-N-vinylcarbazole are prepared by the methods described in U.S. Pat. No. 3,421,891. Nitrated poly-N-vinylcarbazole is prepared by the method described in U.S. Pat. No. 3,418,116. Other polymers are prepared by well-known methods.

For the preparation of the photoconductive insulating layers, a solution of the photoconductive polymer and the sensitizer in a suitable solvent is applied to the supports in the usual manner, for example, spraying, blade coating, wire-rod

coating or whirler coating, and then dried so as to produce a homogeneous photoconductive insulating layer on the electroconductive support. Suitable solvents are benzene, toluene, chlorobenzene, dioxane, methylene chloride, dichloroethane and combinations thereof. The solution may include suitable plasticizers and/or organic colloids for improving the flexibility and strength of the photoconductive compound layer. Suitable plasticizers include chlorinated diphenyl, dimethyl phthalate, diethyl phthalate and octyl phthalate. Suitable organic colloids include natural and synthetic resins, e.g. phenol resin, phenol resin modified with rosin, polyvinyl acetal, polyvinyl butyral, polyvinyl cinnamate and polycarbonate resin. Suitable materials for a conductive support layer are those materials which satisfy the requirement of the electrophotographic art and include metal plates, glass plates having NESA coating and plates or foils made of electrically conductive resins or coated with a vacuum-deposited thin metal layer. Transparent supports can be used to form transparent electrophotographic plates, foils or films.

The reproduction of images by electrophotographic methods is carried out as follows: when the photoconductive insulating layer has been charged by means of a corona discharge apparatus, the electrophotographic material with the photoconductive insulating layer is exposed to light under a master and is then dusted over in a known manner with a resin powder colored with carbon black. The image that now becomes visible can easily be wiped off. It can also be fixed by heating at about 120° C. From positive masters, positive images exhibiting good contrast are produced.

#### EXAMPLE

This invention is still further illustrated with reference to the following examples which are given by way of illustration only.

#### EXAMPLE 1

One gram of poly-N-vinylcarbazole, 0.004 gram of a sensitizer listed in table 3 and 0.5 gram of chlorinated diphenyl (commercially available as "Kanechlor") are dissolved in 10 milliliters of 1,2-dichloroethane. The solution is applied to an aluminum plate and is dried to form a layer 10 $\mu$  in thickness. After the aluminum plate provided with the layer is charged positively by means of corona discharge with a charging device maintained at approximately 6,000 volts in the dark, it is placed under a positive master and is exposed to a 100 W tungsten lamp at an illumination of 50 luxes. Subsequently, the plate is powdered over with a developer in a per se known manner. This developed consists of a toner and a carrier. The toner consists of a low melting-point polystyrene, colophony and carbon-black and is mixed with a carrier substance having a nature such that the toner becomes triboelectrically charged with a charge opposite to that produced on the plate. A positive image is produced and is fixed by slight heating. Table 4 shows the optimum amounts of exposure in lux-second units.

It is clear from table 4 and FIGS. 5 and 6 that the sensitizers improve the photoconductivity and the spectrum response of poly-N-vinylcarbazole.

TABLE 4

| Compound No. | Optimum Exposure (lux.sec.) |
|--------------|-----------------------------|
| None         | 20,000                      |
| 26           | 19                          |
| 27           | 24                          |
| 28           | 20                          |
| 29           | 24                          |
| 30           | 24                          |
| 31           | 23                          |
| 32           | 30                          |
| 33           | 20                          |
| 34           | 29                          |
| 35           | 19                          |
| 36           | 25                          |
| 37           | 23                          |
| 38           | 22                          |
| 39           | 15                          |

|    |    |
|----|----|
| 40 | 22 |
| 41 | 23 |
| 42 | 22 |
| 43 | 70 |
| 44 | 32 |
| 45 | 84 |
| 47 | 70 |
| 50 | 32 |

#### EXAMPLE 2

10 One gram of polyacenaphthylene, 0.6 gram of chlorinated diphenyl (commercially available as "Kanechlor") and 0.004 gram of a sensitizer listed in table 3 are dissolved in 10 milliliters of 1,2-dichloroethane. The solution is applied to an aluminum plate and is dried to form a layer 6 $\mu$  in thickness. An 15 electrophotographic image is produced in the same way as that described in example 1. Table 5 shows the optimum amounts of exposure in lux-second units to produce exactly the original images.

TABLE 5

| Compound No. | Optimum Exposure (lux.sec.) |
|--------------|-----------------------------|
| None         | 200,000                     |
| 27           | 52                          |
| 30           | 60                          |
| 34           | 79                          |
| 39           | 56                          |
| 44           | 66                          |
| 50           | 80                          |

#### EXAMPLE 3

35 Two grams of nitrated poly-N-vinylcarbazole (containing nine nitrated carbazole rings per a hundred carbazole rings), 1 gram of chlorinated diphenyl (commercially available as "Kanechlor") and 0.004 gram of a sensitizer listed in table 3 are dissolved in 10 milliliters of 1,2-dichloroethane. The solution is applied to an aluminum plate and is dried to form a layer 12 $\mu$  in thickness. An 40 electrophotographic image is produced in the same way as that described in example 1. Table 6 shows the optimum amounts of exposure in lux-second units to produce exactly the original images.

#### EXAMPLE 6

| Compound No. | Optimum Exposure (lux.sec.) |
|--------------|-----------------------------|
| None         | 16,000                      |
| 18           | 36                          |
| 19           | 21                          |
| 22           | 24                          |
| 25           | 32                          |
| 27           | 13                          |
| 28           | 17                          |
| 30           | 14                          |
| 33           | 17                          |
| 34           | 15                          |
| 39           | 15                          |
| 50           | 19                          |
| 52           | 36                          |

#### EXAMPLE 4

70 Ten grams of brominated poly-N-vinylcarbazole (monobromo-substituted product), 5 grams of polycarbonate resin (commercially available as "Panlite K"), 3 grams of chlorinated diphenyl (commercially available as "Kanechlor") and 0.04 gram of a sensitizer listed in table 3 are dissolved in a solvent containing 80 milliliters of chlorobenzene and 20 milliliters of 1,2-dichloroethane. This solution is applied to an aluminum plate and is dried to form a layer 14 $\mu$  thickness. An 75 electrophotographic image is produced in the same way as that described in example 1. Table 7 shows the optimum

amounts of exposure in lux-second units to produce exactly the original images.

It is clear from table 7 and FIGS. 3 and 4, that the sensitizers improve the photoconductivity and the spectrum response of brominated poly-N-vinylcarbazole.

TABLE 7

| Compound No. | Optimum Exposure (lux.sec) |
|--------------|----------------------------|
| None         | 80,000                     |
| 18           | 56                         |
| 19           | 26                         |
| 20           | 80                         |
| 22           | 30                         |
| 23           | 52                         |
| 24           | 56                         |
| 26           | 15                         |
| 27           | 15                         |
| 27B          | 10                         |
| 27F          | 13                         |
| 27Z          | 14                         |
| 28           | 18                         |
| 29           | 20                         |
| 30           | 15                         |
| 31           | 16                         |
| 32           | 15                         |
| 33           | 17                         |
| 34           | 20                         |
| 35           | 15                         |
| 36           | 15                         |
| 37           | 17                         |
| 38           | 20                         |
| 39           | 16                         |
| 40           | 19                         |
| 41           | 20                         |
| 42           | 18                         |
| 43           | 85                         |
| 44           | 25                         |
| 45           | 58                         |
| 46           | 70                         |
| 47           | 44                         |
| 48           | 70                         |
| 50           | 40                         |
| 51           | 24                         |
| 52           | 40                         |
| 53           | 40                         |
| 54           | 36                         |
| 55           | 36                         |
| 56           | 40                         |
| 57           | 60                         |
| 58           | 65                         |
| 59           | 25                         |
| 60           | 32                         |
| 61           | 75                         |
| 62           | 90                         |

## EXAMPLE 5

One gram of poly-3,6-dibromo-N-vinylcarbazole, 0.4 gram of chlorinated diphenyl (commercially available as "Kanechlor") and 0.004 gram of a sensitizer listed in table 3 are dissolved in 10 milliliters of 1,2-dichloroethane. The solution is applied to an aluminum plate and is dried to form a layer 8 $\mu$  in thickness. An electrophotographic image is produced in the same way as that described in example 1. Table 8 shows the optimum amounts of exposure in lux-second units to produce exactly the original images.

TABLE 8

| Compound No. | Optimum Exposure (lux.sec) |
|--------------|----------------------------|
| None         | 5,000                      |
| 19           | 21                         |
| 20           | 22                         |
| 24           | 23                         |
| 26           | 9                          |
| 27           | 9                          |
| 28           | 10                         |

31  
37  
42  
59  
11  
11  
10  
13

Applicants' preferred sensitizing compounds are those selected from the reaction products of a benzopyrylium salt having the chemical formula



wherein R<sub>1</sub> is a radical selected from the group consisting of  $\alpha$ -isopropyl- $\omega$ -phenylbutadienyl, methoxystyryl, methoxyphenyl, styryl,  $\alpha$ -isopropyl methoxystyryl,  $\alpha$ -isopropylstyryl and phenyl,  
20 R<sub>2</sub> is hydrogen or phenyl,  
R<sub>3</sub> is hydrogen or methoxy,  
and the anion is selected from the group consisting of  
25 fluoroborate, chloroferrate, chlorozincate and perchlorate anions, with a benzopyran having the chemical formula



35 wherein R<sub>4</sub> is a radical selected from the group consisting of styryl, methoxystyryl,  $\alpha$ -isopropyl- $\omega$ -phenylbutadienyl,  $\alpha$ -isopropyl-methoxystyryl, phenyl,  $\alpha$ -isopropyl styryl and methoxyphenyl,  
R<sub>5</sub> is hydrogen or phenyl, and  
40 R<sub>6</sub> is hydrogen or methoxy.  
What is claimed is:  
1. An electrophotographic material comprising a conductive support layer and a photoconductive insulating layer, the latter comprising a combination of an organic photoconductive compound and a sensitizer, said organic photoconductive compound consisting essentially of at least one compound selected from the group consisting of poly-N-vinylcarbazole, poly-3,6-dibromo-N-vinylcarbazole, brominated poly-N-vinylcarbazole, nitrated poly-N-vinylcarbazole and 45 polyacenaphthylene, said sensitizer comprising a compound selected from the group consisting of reaction products of a benzopyrylium salt having the chemical formula



60 wherein R<sub>1</sub> is a radical selected from the group consisting of  $\alpha$ -isopropyl- $\omega$ -phenylbutadienyl, methoxystyryl, methoxyphenyl, styryl,  $\alpha$ -isopropyl methoxystyryl,  $\alpha$ -isopropylstyryl and phenyl,  
R<sub>2</sub> is hydrogen or phenyl,  
R<sub>3</sub> is hydrogen or methoxy,  
and the anion is selected from the group consisting of  
65 fluoroborate, chloroferrate, chlorozincate and perchlorate anions, with a benzopyran having the chemical formula



wherein  $R_4$  is a radical selected from the group consisting of styryl, methoxystryl,  $\alpha$ -isopropyl- $\omega$ -phenylbutadienyl,  $\alpha$ -isopropyl-methoxystyryl, phenyl,  $\alpha$ -isopropyl styryl and methoxyphenyl,

$R_5$  is hydrogen or phenyl, and

$R_6$  is hydrogen or methoxy.

2. The electrophotographic material of claim 1 wherein the sensitizer is the reaction product of 2-( $\alpha$ -isopropyl- $\omega$ -phenylbutadienyl)-benzopyrylium perchlorate and 2-(p-methoxystyryl)-3-phenyl-4-methoxypyran.

3. The electrophotographic material of claim 1 wherein the sensitizer is the reaction product of 2-(p-methoxystyryl)-3-phenyl-benzopyrylium perchlorate and 2-(p-methoxystyryl)-3-phenyl-4-methoxypyran.

4. The electrophotographic material of claim 1 wherein the

sensitizer is the reaction product of 2-(p-methoxylphenyl)-benzopyrylium perchlorate and 2-(p-methoxystyryl)-3-phenyl-4-methoxypypane.

5. The electrophotographic material of claim 1 wherein the sensitizer is the reaction product of 2-styryl-3-phenylbenzopyrylium perchlorate and 2-styryl-3-phenyl-4-methoxybenzopyrane.

6. The electrophotographic material of claim 1 wherein the sensitizer is the reaction product of 2-phenylbenzopyrylium perchlorate and 2-phenyl-4-methoxybenzopyrane.

7. The electrophotographic material of claim 1 wherein the sensitizer is the reaction product of 2-(p-methoxyphenyl)benzopyrylium perchlorate and 2-(p-methoxyphenyl)-4-methoxybenzopyrane.

\* \* \* \* \*

20

25

30

35

40

45

50

55

60

65

70

75